

## UNITED STATES PATENT OFFICE

1,975,375

## ALLOY

Georg Schichtel, Dobriach on Millstattersee, Austria, assignor to American Magnesium Metals Corporation, Pittsburgh, Pa., a corporation of Delaware

No Drawing. Original application November 18, 1932, Serial No. 643,297. Divided and this application August 22, 1933, Serial No. 686,319. In Austria February 19, 1932

3 Claims. (Cl. 75—1)

This application is a division of my prior application Serial No. 643,297, filed November 18, 1932.

The present improved alloy is one in which magnesium is the predominant element, the primary object being to develop an alloy that will possess the characteristic low specific gravity which is obtained by the use of magnesium in excess of 80 per cent while such alloy will be characterized by higher resistance to corrosion and at the same time will have a higher strength than the known alloys of this kind.

The known alloys in use containing generally more than 85% magnesium and as principal 15 additional ingredient aluminum or zinc or both of these ingredients, other constituents being present in relatively small amounts, do not exhibit a sufficient resistance to corrosion by water or even by damp air, and cannot be used at all 20 when in continuous contact with sea-water. Various attempts have been made to render the surfaces of these metals more resistant by applying coatings, but such attempts failed since corrosion often takes place to an increased extent 25 when the superficial protective layer is damaged.

The object of the invention is attained by the addition of further additional metals to the alloys, namely antimony or bismuth or both of these metals amounting in general to not less 30 than 0.05% and not more than 2% of the total.

The most diverse alloys of the kind referred to containing antimony or bismuth have proved distinctly superior, when exposed to the action of a 3% solution of common salt, to alloys of the 35 same kind which do not contain antimony or bismuth; whilst the alloys containing antimony or bismuth showed an almost unaltered surface, the samples devoid of antimony or bismuth were strongly corroded on carrying out the comparative tests.

In general the lower limit of efficiency is given by additions of 0.05%, and it is preferable not to exceed the upper limit of 2%.

From their position in the electrochemical 45 series antimony and bismuth are more valuable than magnesium, and moreover do not form a solid solution with the latter; the assumption therefore would rather have been that the addition of these metals to the known alloys of magnesium would involve decreasing their resistance to corrosion.

The magnesium-base alloys developed by the present invention show also a considerable increase in strength, without the elongation decreasing. As the magnesium alloys of the kind

hitherto in use (electron, Dow-metal) have a comparatively small strength, this constitutes a further advance of considerable importance, the more so as the specific gravity of the alloys is scarcely increased to any perceptible extent by 60 the small amount of the added metals.

Furthermore, the alloys according to the invention show in comparison with similarly composed known electron alloys an increase of the permanent impact strength by 50%. 65

The alloys may be used as cast alloys or mechanically worked alloys and may be improved by thermal treatments.

A satisfactory formula for an alloy according to my invention, in which zinc is the principal 70 additional ingredient is as follows, viz:—

Magnesium 94.7%, zinc 4.3%, antimony 1%;  
Magnesium 96.2%, zinc 3.5%, bismuth 0.3%.

What I claim is:—

1. A low specific gravity magnesium-base alloy 75 containing from about 80% to 98.9 percent of magnesium, and zinc in an amount between about 1 to about 20%, and subject to corrosion, this alloy being rendered more resistant against corrosion by the addition of at least one metal 80 of the group consisting of antimony and bismuth in an amount from 0.05 to 2%.

2. A low specific gravity magnesium-base alloy consisting of from about 86% to 98.8% of magnesium, from about 1 to 10% of zinc, and 85 from about 0.05 to 2% of at least one metal of the group consisting of antimony and bismuth.

3. A low specific gravity magnesium-base alloy consisting of from about 86 to 98.8% of magnesium, from about 1 to about 10% of zinc, and 90 antimony and bismuth in a combined amount of from about 0.05 to 2%. 95

GEORG SCHICHTEL.

95

100

105

110